

1

2,920,949

**PROCESS OF PRODUCING AN INCENDIARY COMPOSITION**

Morris S. Kharasch, Chicago, Ill., assignor to the United States of America as represented by the Secretary of War

No Drawing. Application December 30, 1943  
Serial No. 516,313

3 Claims. (Cl. 52—23)

The invention described herein may be manufactured and used by or for the Government for governmental purposes without the payment to me of any royalty thereon.

This invention relates particularly to an incendiary agent adapted for use in pyrotechnical devices, such as incendiary grenades and bombs. It is concerned particularly with the use of polymers of acetylenes as incendiary agents.

Upon investigation of low molecular weight acetylene compounds, such as divinyl acetylene, a by-product in the manufacture of chloroprene rubber, it was found that there was little likelihood of using such a compound directly as an incendiary agent, because in the first place such substances are highly volatile, and in the second place they quickly absorb oxygen to form peroxides which explode violently on the slightest touch. However, I have discovered that polymerized derivatives of acetylenes have properties which adapt them for use as incendiary agents.

An object of this invention is to utilize suitably stable polymers of acetylenes including copolymers, particularly polymers of divinyl acetylene and the like, as incendiary agents.

Another object of this invention is to provide a process for forming solid incendiary materials comprising polymers of acetylenes.

A further object of this invention is to provide useful warfare munitions comprising incendiary agents in which suitable polymers of acetylenes are utilized.

It has now been found that there are derivatives of acetylene, particularly vinyl acetylenes, which are very suitable for use as incendiary agents. One of these derivatives is polymerized divinyl acetylene. This substance which comprises principally the trimer with some tetramer can be available in fairly large quantities as an industrial by-product. It has been commercially sold as an 80% solution in toluene or xylene. It is used as an acid-proof coating for materials. This material, when properly handled, is not unduly hazardous. It does not ignite too readily and burns with a smoky flame. Nevertheless, it has been possible to adopt this substance as an organic component of a very effective incendiary material which has proved to be of considerable interest as fillers for grenades.

The incendiary substances containing polymers may also be used to fill large incendiary munitions, such as bombs; and they have proved to be useful as binders for propellants.

There are two types of grenades or hand incendiaries in which the acetylenic polymer incendiary compositions have been found to be very effective. They are paper tubes and magnesium tubes with the incendiary agent compressed therein. In both types, a button of match-head composition was attached to one end of the tube, this end being closed with a removable cap coated with a friction material. The finished incendiary resembled in outward appearance a shortened railway fuze. It was

2

easily ignited by striking the match-head with the removable cap. Hand incendiaries of this type with total weights of 90 to 250 grams were subjected to tests. The sizes mentioned are arbitrary, for tubes of any size can be filled with the incendiary agent.

5 The distinguishing characteristics of these incendiaries are as follows: they burn with a vigorous torch-like flame which extends a foot or more from the mouth of the tube. The burning polymer incendiary agent ignites magnesium; and when magnesium tubes are used, much longer flames are often obtained during the time when the polymer incendiary agent and magnesium are burning simultaneously.

10 The polymer incendiaries were tested on wooden attic-type structures. In all instances, they were at least as effective as any other type of incendiary tested in producing sustaining fires; i.e., fires which cause complete conflagration of a structure.

15 If the incendiary tubes or containers for the acetylene polymer agent are coated on the outside with paraffin, 20 they may be soaked for several hours in water without impairing either their ignition or their burning properties.

25 In comparison with hand incendiaries using thickened kerosene in Celluloid containers, acetylenic polymer incendiaries have the following advantages: they are hard tubes filled with a solid; hence, they cannot be crushed readily and contain no liquid to escape from a damaged container. As long as the igniting agent or match-head composition is not exposed, it is almost impossible to ignite the incendiary with a match or cigarette. The vigorous flame produced by the acetylene polymer incendiary agent is but little affected by wind.

30 For the purpose of illustration, the following example is given on the preparation of a solid acetylene polymer incendiary agent:

*Example*

35 A mixture is prepared to contain about 30% of an 40 80% solution of divinyl acetylene polymer in an aromatic hydrocarbon, about 10% heavy petroleum oil and about 60% crude sodium nitrate; and the liquid divinyl acetylene polymer is then further polymerized by heating the mass to 85° C. in air for about 16 hours. A solid mass thus formed is rolled to produce a uniform granular 45 material. The product is stable and can at any time be loaded into tubes, for example, using a pressure of about 2,000 lbs. per square inch.

50 For a given acetylene polymer mixture, the burning time of the incendiaries thus prepared is proportional to the length of the tube and, within wide limits, dependent on the cross section. The burning rate varies somewhat with the quantity of heavy oil used and with the mesh and nature of the oxidizing salt; of these, the latter is the 55 more important. By controlling these factors, there have been prepared 7-inch incendiaries having combustion periods varying from about 1½ to 6 minutes.

56 The magnesium tubing used in some of the hand incendiaries submitted for test had a wall thickness of  $\frac{3}{32}$  inch. Each tube was one inch in diameter and 6½ inches 60 long; the filled tubes weighed about 190 grams. The polymerized acetylene agent burned for about 1 to 1½ minutes before the magnesium tubing ignited. The magnesium and the filling then burned together, and a vigorous burning of the magnesium took place in less than another minute. There was further burning which lasted for several minutes. It was found possible to vary, under wide limits, the time before the ignition of the magnesium casing and the time during which this casing burns 65 vigorously, particularly by varying the mesh of the nitrate and the type of the oxidizing agent. For maximum effect, it is advantageous to have the magnesium burn rapidly.

7-inch incendiaries in paper tubes which were submitted to tests burned for about three minutes.

The acetylenes from which the incendiary agents are derived are highly unsaturated aliphatic hydrocarbons, typified by acetylene,  $\text{CH} \equiv \text{CH}$ ; acetylene tetramer,



and the resembling divinyl acetylene



The derivatives that may be used include polymers, copolymers with other acetylenes or other types of hydrocarbons, metallic derivatives and other substitution or addition products.

The polymerized acetylenes may be used in mixtures and in conjunction with other incendiary agents, such as thickened gasoline, Thermit type agents, phosphorus, granular magnesium and the like. They may be used with various types of oxidizing agents, stabilizing agents, also with starting and igniting agents generally employed for incendiaries.

It is to be understood that the invention is not to be limited by the specific illustrative examples and that modifications come within the spirit and scope of the invention.

I claim:

1. A process for producing an incendiary material

comprising preparing a mixture of about 30% of an 80% solution of the polymer of divinyl acetylene in an aromatic hydrocarbon, about 10% heavy mineral oil and about 60% sodium nitrate, exposing said mixture to air until a solid mass adapted to be crumbled is formed, and then rolling said mass, until the mixture is uniformly granulated.

2. The process of claim 1 in which the temperature of the air is maintained at approximately 85° C.

3. The process of claim 1 in which said air is maintained at a temperature of approximately 85° C. and the granular mixture is finally compressed by a pressure of about 2000# per square inch.

15 References Cited in the file of this patent

UNITED STATES PATENTS

|           |           |                |
|-----------|-----------|----------------|
| 1,361,286 | Patrick   | Dec. 7, 1920   |
| 1,436,248 | Hammond   | Nov. 21, 1922  |
| 1,812,541 | Nieuwland | June 30, 1931  |
| 1,896,162 | Carter    | Feb. 7, 1933   |
| 2,294,415 | McBride   | Sept. 1, 1942  |
| 2,329,522 | Duncan    | Sept. 14, 1943 |

20 FOREIGN PATENTS

|    |         |               |              |
|----|---------|---------------|--------------|
| 25 | 127,050 | Great Britain | May 29, 1919 |
|----|---------|---------------|--------------|